

1

3,457,185

**CORROSION INHIBITED ACIDIC SOLUTIONS  
CONTAINING ALKYL HEXAHYDROPRIMIDINE-2-THIONE AND QUATERNARY AMMONIUM COMPOUNDS**

Roy J. Betty and Robert E. Malec, Chicago, Ill., and Charles E. Tippett, Dayton, Ohio, assignors, by mesne assignments, to Armour Industrial Chemical Company, a corporation of Delaware  
No Drawing. Filed Oct. 14, 1966, Ser. No. 586,667  
Int. Cl. C23f 11/04, 11/10, 11/14  
U.S. Cl. 252—391 10 Claims

**ABSTRACT OF THE DISCLOSURE**

Corrosion inhibiting compositions comprising either N-aliphatic hexahydropyrimidine-2-thione having an alkyl radical containing from 6-22 carbon atoms, or a combination of said thione and a quaternary ammonium compound; and a process for protecting metals in contact with corroding aqueous acidic solutions employing from 10 to 50,000 p.p.m. of such compositions.

This invention relates to new corrosion inhibitor compositions and to a process for protecting metals in contact with corroding aqueous acidic solutions. More particularly it relates to long chain N-aliphatic hexahydropyrimidine thiones in aqueous solutions of acids to inhibit the corrosion of metals in contact with such solutions.

It is well known that the corrosion of metallic substances by the action of aqueous acids such as sulfuric, hydrochloric, phosphoric, sulfamic and citric is a serious problem to industry. This problem is generally experienced in chemical and electrolytic pickling operations wherein baths of aqueous acid solutions are used to remove oxides, carbonates or other scales from metals. It is also experienced in aqueous dipping processes; in plant "washout" procedures to clean equipment such as industrial boilers, condensers, heat exchangers and the like with a variety of dilute aqueous acid solutions; in petroleum well operations; and in the storage and handling of aqueous acids and acid containing solutions. A particularly difficult handling and storage problem is encountered with concentrated phosphoric acid to be used in the manufacture of liquid fertilizers.

It is also known that corrosion inhibitors generally have limited application due to the widely different character of the conditions present in each situation where acid corrosion of metal is a problem. Thus the search for better corrosion inhibitors in a particular area must necessarily be conducted largely on an empirical basis.

It was therefore surprising to discover a class of corrosion inhibitor compositions which are highly effective under widely varying conditions of use. In one of its aspects this invention relates to corrosion inhibited acidic solutions comprising N-aliphatic hexahydropyrimidine-2-thiones useful in the cleaning of metallic surfaces. In another of its aspects, this invention relates to corrosion inhibited acidic solutions useful in the manufacture of liquid fertilizers. In still another of its aspects, this in-

2

vention relates to corrosion inhibited acidic solutions useful in the storage and transporting of aqueous acids in general.

It is therefore an object of this invention to provide a process for protecting metals from corrosion by aqueous acidic solutions under varying conditions of use.

Another object of this invention is to provide corrosion inhibitor compositions for use in the process of this invention.

Still another object of this invention is to provide corrosion inhibitor compositions in which the solubilizing agent for the corrosion inhibitor cooperates with the inhibitor to increase its effectiveness in protecting metal surfaces.

A further object of this invention is to provide corrosion inhibitor compositions for use in the process of this invention which are effective to inhibit acid corrosion of non-ferrous metals as well as ferrous metals and do not substantially stain the metals to be protected.

Other objects and advantages and a fuller understanding of this invention will become apparent from the ensuing description and examples.

In British Patent No. 1,067,399 granted Aug. 23, 1967, there is described a method for the manufacture of long chain N-alkyl hexahydropyrimidine-2-thiones. In the manner therein described it is possible to obtain compounds of the following structure which we have discovered can be used to effectively inhibit the corrosion of metal by aqueous acidic solutions and to substantially accomplish the objects and aspects of this invention set out above. The formula of the N-aliphatic hexahydropyrimidine-2-thiones useful to this invention is as follows:



wherein R is an aliphatic hydrocarbon radical having from 6 to 22 carbon atoms. Within the meaning of our invention, R may be a straight or branched chain, saturated or unsaturated aliphatic hydrocarbon radical.

In accordance with our invention, it has been found that the corrosive tendencies of aqueous solutions of acid such as sulfuric, hydrochloric, phosphoric, sulfamic and citric may be substantially reduced or mitigated by incorporating into such acids a corrosion-inhibiting amount of certain N-aliphatic hexahydropyrimidine-2-thiones either alone or with known corrosion inhibitors such as a quaternary ammonium compound, and thereafter causing the aqueous acidic solution to contact the metal to be protected.

The amount of inhibitor necessary in a particular acidic system to obtain optimum inhibition will depend upon environmental circumstances such as the particular metallic substance, the particular acid present in the aqueous corroding solution, the concentration of the acid, and the temperature at which the system is maintained. Generally, we use a concentration range of 10 to 50,000 parts of inhibitor per million parts of aqueous acidic

solution. Our preferred range is 50 to 200 parts per million.

The temperatures of metal corroding aqueous acid systems are quite often found to be in excess of 100° F. and may be as high as 210° F. The concentrations of the acids encountered may be as varying as from .01% to 80% by weight. As would be expected, where the concentration of the acid employed is high and the temperature is elevated, a larger quantity of inhibitor will be required than when lower temperatures and more dilute solutions of acid are employed, wherein the concentration of the inhibitor to produce substantial inhibition of metal corrosion may be proportionately reduced. The N-aliphatic hexahydropyrimidine-2-thiones useful in our process may be added to an aqueous acidic media to inhibit corrosion of metals contacting the media either singularly, in combination with other of the desirable N-aliphatic hexahydropyrimidine-2-thiones or in combination with known inhibitors. In general, economics will govern the quantity of inhibitor or inhibitor mixtures to be added to any particular system and only that quantity of the inhibitor composition which will produce the result desired will be introduced into the particular system.

In the practice of our invention where ferrous metallic substances are to be contacted by corroding acid media, we prefer to add a corrosion inhibiting composition comprising N-(C<sub>7</sub>-C<sub>9</sub> sec-alkyl)-hexahydropyrimidine-2-thione and 15% by weight or less of the particular acid such as sulfuric, hydrochloric, phosphoric, sulfamic or citric. This composition does not substantially stain the metal. A particularly useful corrosion inhibitor composition for ferrous metallic substances contacted by phosphoric acid systems containing up to about 80% by weight phosphoric acid or the salts thereof is the mixture of (A) N-(C<sub>7</sub>-C<sub>9</sub> sec-alkyl)-hexahydropyrimidine-2-thione and (B) as a solubilizing substance or agent, a quaternary ammonium compound of the formula R<sub>1</sub>R<sub>2</sub>R<sub>3</sub>R<sub>4</sub>NX wherein R<sub>1</sub> is an aliphatic hydrocarbon radical containing from 6 to 22 carbon atoms, R<sub>2</sub> is an alkyl radical containing from 1 to 3 carbon atoms, R<sub>3</sub> is a hydrocarbon radical selected from the group consisting of R<sub>1</sub>, R<sub>2</sub> and (R'O)<sub>x</sub>H wherein R' is an alkylene radical having between 2 and 3 carbon atoms, R<sub>4</sub> is a hydrocarbon radical selected from the group consisting of R<sub>1</sub>, R<sub>2</sub> and (R'O)<sub>y</sub>H provided that when R<sub>3</sub> is (R'O)<sub>x</sub>H, R<sub>4</sub> is (R'O)<sub>y</sub>H and x and y are integers having a sum between 2 and 50, and X is a halogen. R<sub>1</sub> within the above definition may be straight or branched chain, saturated or unsaturated aliphatic hydrocarbon.

A typical group of commercially available quaternary ammonium compounds that are within the above definition and are suitable for use in our compositions and process have the trademark Arquad and are manufactured by Armour Industrial Chemical Company, a division of Armour and Company. Preferred quaternary ammonium compounds include:

N-coco-N,N,N-trimethyl ammonium chloride (50% active), the symbol coco standing for a mixture of long chain hydrocarbon radicals derived from coconut oil. N,N-dicoco-N,N-dimethyl ammonium chloride (75% active).

N,N-di(di-hydroxy tallow) - N,N - dimethyl ammonium chloride (75% active), the symbol tallow standing for a mixture of long chain hydrocarbon radicals derived from tallow.

N-(C<sub>11</sub>-C<sub>14</sub> sec-alkyl)-N,N,N-trimethyl ammonium chloride.

N-(C<sub>14</sub>C<sub>19</sub> sec-alkyl)-N,N,N-trimethyl ammonium chloride.

Another suitable group of quaternary ammonium compounds within the above definition is an ethoxylated quaternary ammonium salt of the trademark Ethoquad manufactured by Armour Industrial Chemical Company. A preferred ethoxylated quaternary ammonium salt is

N - methyl - N - coco - N,N - polyethyleneoxide (15 moles) ammonium chloride.

No special conditions are necessary to form the inhibitor compositions of a N-(sec-alkyl)-hexahydropyrimidine-2-thione plus a quaternary ammonium compound. One component of the mixture is merely added to the other in the desired proportions. Suitable proportions may be obtained with about 25% to about 75% by weight of the N-(sec-alkyl)-hexahydropyrimidine - 2 - thione in combination with about 75% to about 25% by weight of the solubilizing agent. Our preferred ratio by weight is about 40 to 60% of the N-(sec-alkyl)-hexahydropyrimidine-2-thione to about 60 to 40% of the solubilizing agent. As with the use of the N-aliphatic hexahydropyrimidine-2-thiones alone or in combination with each other or known corrosion inhibitors, the amount of the N-(sec-alkyl) - hexahydropyrimidine - 2 - thione and quaternary ammonium compound corrosion inhibitor compositions which should be incorporated into a particular aqueous acid containing system in order to achieve a metal corrosion inhibiting result can be varied widely and is largely dependent upon the concentration of the acid in the system. A result has been obtained with an effective amount more than 50 parts per million by weight of these compositions, but the preferred concentration range is 100 to 400 parts per million. In general, economics will govern and only that amount of the compositions which will produce the result desired will be introduced into a particular system. Our N - (sec - alkyl) - hexahydropyrimidine - 2 - thione and quaternary ammonium compound compositions are liquid at room temperatures and are very readily soluble in aqueous acid systems containing a high concentration of phosphoric acid or salts thereof. The compositions, further, do not degrade in such systems and therefore will not leave a residue in the treated system. In addition the compositions, when added to aqueous acid solutions will not substantially stain the metal to be protected.

In order to more fully understand the nature of the compositions of the present process, their characteristics, and the manner in which they may be used, the following illustrative specific examples are provided. The parts used are expressed as percent by weight in the total aqueous mixture unless otherwise specified.

#### EXAMPLE I

50 N - (C<sub>7</sub>-C<sub>9</sub> sec - alkyl) - hexahydropyrimidine - 2 - thione, N - octyl - hexahydropyrimidine - 2 - thione and N - dodecylhexahydropyrimidine - 2 - thione were tested for corrosion inhibition of 1020 mild steel in contact with aqueous sulfuric acid as follows:

55 A series of 8 oz. bottles containing 150 ml. of acid solution and a quantity of the corrosion inhibitor were placed in an oil bath. The coupons of 1020 mild steel, approximately 1" x 3" x .036" were cleaned in the following manner before initial weighings: they were tumble in a ball mill with alumnum powder, removed, dipped in hot isopropyl alcohol, then dipped in hot acetone, and air dried. The pre-weighed coupons were submerged in the acid-inhibitor solutions and maintained there at 200° F. for 6 hours. Upon completion of the time period, the coupons were removed (rinsed in hot water and 60 dipped in hot isopropyl alcohol and then in hot acetone, then air dried and reweighed. The concentrations of the acid used were on a weight basis, and the percent inhibitor was based on the weight of the total solution. These are shown in Table I. For comparison, no inhibitor was 65 added in certain instances and this fact is shown in Table I. Certain known inhibitors were also run under the same conditions and they are identified in Table I. Corrosion rates were calculated on a weight loss basis and expressed in pounds per square foot per day (lb./ft.<sup>2</sup>/day). 70 The results of the tests are set forth in Table I.

TABLE I

| Inhibitor                                                                      | Percent H <sub>2</sub> SO <sub>4</sub> | Percent Inhibitor | Corrosion Rate (lb./ft. <sup>2</sup> /day) |
|--------------------------------------------------------------------------------|----------------------------------------|-------------------|--------------------------------------------|
| None                                                                           | 15                                     | —                 | (i)                                        |
| N-(C <sub>7</sub> -C <sub>9</sub> sec-alkyl)-hexahydro-<br>pyrimidine-2-thione | 15                                     | .01               | .0201                                      |
| Do                                                                             | 15                                     | .03               | .0160                                      |
| Do                                                                             | 15                                     | .04               | .0191                                      |
| Do                                                                             | 15                                     | .05               | .0188                                      |
| Do                                                                             | 15                                     | .06               | .0179                                      |
| N-octyl-hexahydro-<br>pyrimidine-2-thione                                      | 15                                     | .03               | .0302                                      |
| N-dodecyl-hexahydro-<br>pyrimidine-2-thione                                    | 15                                     | .03               | .7768                                      |
| Diethyl thiourea                                                               | 15                                     | .03               | .0790                                      |
| Do                                                                             | 15                                     | .06               | .0232                                      |
| Propylene thiourea                                                             | 15                                     | .01               | 1.6973                                     |
| Do                                                                             | 15                                     | .03               | .1675                                      |
| Do                                                                             | 15                                     | .05               | .2655                                      |
| Ethylene thiourea                                                              | 15                                     | .01               | 1.6139                                     |
| Do                                                                             | 15                                     | .03               | .9763                                      |
| Do                                                                             | 15                                     | .05               | .2073                                      |
| None                                                                           | 20                                     | —                 | (i)                                        |
| N-(C <sub>7</sub> -C <sub>9</sub> sec-alkyl)-hexahydro-<br>pyrimidine-2-thione | 20                                     | .006              | .1534                                      |
| Do                                                                             | 20                                     | .008              | .1141                                      |
| Do                                                                             | 20                                     | .01               | .0275                                      |
| Do                                                                             | 20                                     | .03               | .0193                                      |
| Do                                                                             | 20                                     | .05               | .0164                                      |
| None                                                                           | 25                                     | —                 | (i)                                        |
| N-(C <sub>7</sub> -C <sub>9</sub> sec-alkyl)-hexahydro-<br>pyrimidine-2-thione | 25                                     | .01               | .1217                                      |
| Do                                                                             | 25                                     | .02               | .0265                                      |
| Do                                                                             | 25                                     | .03               | .0216                                      |
| Do                                                                             | 25                                     | .04               | .0234                                      |
| Do                                                                             | 25                                     | .05               | .0243                                      |

<sup>1</sup> Coupon completely dissolved.

## EXAMPLE II

Coupons of 1020 mild steel were placed as described in Example I in bottles containing 15% sulfuric acid and an inhibitor and then maintained at 200° F. for 6 hours for the tests. The inhibitors tested were N-(C<sub>9</sub>-C<sub>11</sub> sec-alkyl)-hexahydro-  
pyrimidine-2-thione, N-(C<sub>11</sub>-C<sub>14</sub> sec-alkyl)-hexahydro-  
pyrimidine-2-thione, and N-(C<sub>15</sub>-C<sub>20</sub> sec-alkyl)-hexahydro-  
pyrimidine-2-thione. The percent by weight of the inhibitor compositions and the results of the tests are shown in Table II.

TABLE II

| Inhibitor                                                                        | Percent H <sub>2</sub> SO <sub>4</sub> | Percent Inhibitor | Corrosion Rate (lb./ft. <sup>2</sup> /day) |
|----------------------------------------------------------------------------------|----------------------------------------|-------------------|--------------------------------------------|
| None                                                                             | 15                                     | —                 | 2.58                                       |
| N-(C <sub>9</sub> -C <sub>11</sub> sec-alkyl)-hexahydro-<br>pyrimidine-2-thione  | 15                                     | .02               | 0.0238                                     |
| Do                                                                               | 15                                     | .03               | 0.0225                                     |
| Do                                                                               | 15                                     | .04               | 0.0236                                     |
| N-(C <sub>11</sub> -C <sub>14</sub> sec-alkyl)-hexahydro-<br>pyrimidine-2-thione | 15                                     | .02               | 0.0360                                     |
| Do                                                                               | 15                                     | .03               | 0.0272                                     |
| Do                                                                               | 15                                     | .04               | 0.0238                                     |
| N-(C <sub>15</sub> -C <sub>20</sub> sec-alkyl)-hexahydro-<br>pyrimidine-2-thione | 15                                     | .02               | .368                                       |
| Do                                                                               | 15                                     | .03               | .426                                       |
| Do                                                                               | 15                                     | .04               | .594                                       |

## EXAMPLE III

Coupons of stainless steel were placed as described in Example I in bottles containing 15% sulfuric acid and N-(C<sub>7</sub>-C<sub>9</sub> sec-alkyl)-hexahydro-  
pyrimidine-2-thione and there maintained at 200° F. for the times as shown in Table III. As one skilled in the art will recognize, the build-up of a layer of scale or corrosion upon a metal surface will partially protect the metal surface underneath from further corrosion; thus a greater weight loss by acid corrosion will occur in a short period of time than occurs in a longer period of time. This phenomenon may be observed in the results of this test, shown in Table III, and it, along with the different types of stainless steel used, accounts for the increased corrosion rates at 2 and 3 hours as compared with 6 hours.

TABLE III

| Inhibitor                                                                      | Type of Stainless Steel | Hours | Percent Inhibitor | Corrosion Rate (lb./ft. <sup>2</sup> /day) |
|--------------------------------------------------------------------------------|-------------------------|-------|-------------------|--------------------------------------------|
| None                                                                           | 316                     | 6     | —                 | 0.0761                                     |
| N-(C <sub>7</sub> -C <sub>9</sub> sec-alkyl)-hexahydro-<br>pyrimidine-2-thione | 316                     | 6     | .01               | .0016                                      |
| Do                                                                             | 316                     | 6     | .02               | .0013                                      |
| None                                                                           | 410                     | 3     | —                 | 5.6308                                     |
| N-(C <sub>7</sub> -C <sub>9</sub> sec-alkyl)-hexahydro-<br>pyrimidine-2-thione | 410                     | 3     | .01               | 4.4983                                     |
| Do                                                                             | 410                     | 3     | .02               | 0.3274                                     |
| Do                                                                             | 410                     | 3     | .03               | .1572                                      |
| Do                                                                             | 410                     | 3     | .04               | .0856                                      |
| None                                                                           | 420                     | 2     | —                 | 2.5627                                     |
| N-(C <sub>7</sub> -C <sub>9</sub> sec-alkyl)-hexahydro-<br>pyrimidine-2-thione | 420                     | 2     | .06               | .0493                                      |
| Do                                                                             | 430                     | 2     | .03               | 6.6680                                     |
| N-(C <sub>7</sub> -C <sub>9</sub> sec-alkyl)-hexahydro-<br>pyrimidine-2-thione | 430                     | 2     | .01               | 0.2030                                     |
| Do                                                                             | 430                     | 2     | .03               | .0420                                      |
| Do                                                                             | 430                     | 2     | .06               | .0193                                      |

## EXAMPLE IV

The experimental procedure in this test was the same as that used in Example I. Coupons of 1020 mild steel were placed as described in Example I in bottles containing 15% hydrochloric acid and N-(C<sub>7</sub>-C<sub>9</sub> sec-alkyl)-hexahydro-  
pyrimidine-2-thione and there maintained at 200° F. for 3 hours. The results are shown in Table IV.

TABLE IV

| Inhibitor                                                                      | Percent HCl | Percent Inhibitor | Corrosion Rate (lb./ft. <sup>2</sup> /day) |
|--------------------------------------------------------------------------------|-------------|-------------------|--------------------------------------------|
| None                                                                           | 15          | —                 | (i)                                        |
| N-(C <sub>7</sub> -C <sub>9</sub> sec-alkyl)-hexahydro-<br>pyrimidine-2-thione | 15          | .05               | 0.1565                                     |
| Do                                                                             | 15          | .15               | .1101                                      |
| Do                                                                             | 15          | .30               | .1181                                      |

<sup>1</sup> Coupon completely dissolved.

## EXAMPLE V

The experimental procedure used was the same as that used in Example I. N-(C<sub>7</sub>-C<sub>9</sub> sec-alkyl)-hexahydro-  
pyrimidine-2-thione and different aqueous acids were tested for corrosion inhibition of various metals maintained in the corroding acidic solutions at 200° F. for 6 hours. The results are tabulated in Table V.

TABLE V

| Acid and Percent Acid | Metal               | Percent Inhibitor | Corrosion Rate (lb./ft. <sup>2</sup> /day) |
|-----------------------|---------------------|-------------------|--------------------------------------------|
| Sulfamic 15%          | 1020 Mild Steel     | None              | 1.15                                       |
| Do                    | do                  | .01               | .00954                                     |
| Do                    | do                  | .02               | .00820                                     |
| Do                    | do                  | .03               | .0106                                      |
| Do                    | do                  | .04               | .0124                                      |
| Do                    | do                  | .05               | .0128                                      |
| Do                    | do                  | .06               | .0127                                      |
| Do                    | 316 Stainless Steel | None              | .00845                                     |
| Do                    | do                  | .04               | .00134                                     |
| Do                    | do                  | .05               | .00134                                     |
| Do                    | do                  | .06               | .00136                                     |
| Do                    | 410 Stainless Steel | None              | 1.56                                       |
| Do                    | do                  | .04               | .764                                       |
| Do                    | do                  | .05               | .254                                       |
| Do                    | do                  | .06               | .192                                       |
| Do                    | Aluminum            | None              | .124                                       |
| Do                    | do                  | .04               | .0788                                      |
| Do                    | do                  | .05               | .0830                                      |
| Do                    | do                  | .06               | .0773                                      |
| Do                    | Monel               | None              | .000995                                    |
| Do                    | do                  | .04               | .000908                                    |
| Do                    | do                  | .05               | .000848                                    |
| Do                    | do                  | .06               | .000887                                    |
| Phosphoric 15%        | 1020 Mild Steel     | None              | 1.07                                       |
| Do                    | do                  | .01               | .0056                                      |
| Do                    | do                  | .02               | .0046                                      |
| Do                    | do                  | .03               | .0053                                      |
| Do                    | do                  | .04               | .0093                                      |
| Do                    | do                  | .05               | .0044                                      |
| Do                    | do                  | .06               | .0044                                      |
| Do                    | 316 Stainless Steel | None              | .00005                                     |
| Do                    | do                  | .04               | .000015                                    |
| Do                    | do                  | .05               | .000063                                    |
| Do                    | do                  | .06               | .0000144                                   |
| Do                    | Aluminum            | None              | .538                                       |
| Do                    | do                  | .04               | .500                                       |
| Do                    | do                  | .05               | .481                                       |
| Do                    | do                  | .06               | .496                                       |
| Do                    | Monel               | None              | .00097                                     |
| Do                    | do                  | .04               | .00074                                     |

7  
TABLE V—Continued

| Acid and Percent Acid | Metal               | Percent Inhibitor | Corrosion Rate (lb./ft. <sup>2</sup> /day) |
|-----------------------|---------------------|-------------------|--------------------------------------------|
| Do.                   | do.                 | .05               | .00084                                     |
| Do.                   | do.                 | .06               | .00080                                     |
| Citric 15%            | 1020 Mild Steel     | None              | .286                                       |
| Do.                   | do.                 | .01               | .00352                                     |
| Do.                   | do.                 | .02               | .00279                                     |
| Do.                   | do.                 | .03               | .0034                                      |
| Do.                   | do.                 | .04               | .0034                                      |
| Do.                   | do.                 | .05               | .00332                                     |
| Do.                   | do.                 | .06               | .00364                                     |
| Do.                   | 316 Stainless Steel | None              | .00105                                     |
| Do.                   | do.                 | .04               | .00105                                     |
| Do.                   | do.                 | .05               | .00128                                     |
| Do.                   | do.                 | .06               | .00098                                     |
| Do.                   | Monel               | None              | .00084                                     |
| Do.                   | do.                 | .04               | .00044                                     |
| Do.                   | do.                 | .05               | .00048                                     |
| Do.                   | do.                 | .06               | .00040                                     |

## EXAMPLE VI

Using the experimental procedure as set forth in Example I, tests were run on mixtures of (A) an N-(sec-alkyl)-hexahydropyrimidine-2-thione and (B) N-methyl-N-coco-N,N-polyethylene oxide (15 moles) ammonium chloride, as corrosion inhibiting compositions for 75% phosphoric acid contacting 1020 mild steel coupons. The tests were run at 120° F. for 48 hours. The compositions used and the results of the tests are set forth in Table VI.

TABLE VI

| Inhibitor Composition                                                                                                                              | Percent Inhibitor | Corrosion Rate (lb./ft. <sup>2</sup> /day) |
|----------------------------------------------------------------------------------------------------------------------------------------------------|-------------------|--------------------------------------------|
| N-(C <sub>9</sub> -C <sub>11</sub> sec-alkyl)-hexahydropyrimidine-2-thione and N-methyl-N-coco-N,N-polyethyleneoxide (15 moles) ammonium chloride  | .03               | 0.059                                      |
| N-(C <sub>11</sub> -C <sub>13</sub> sec-alkyl)-hexahydropyrimidine-2-thione and N-methyl-N-coco-N,N-polyethyleneoxide (15 moles) ammonium chloride | .03               | 0.022                                      |
| N-(C <sub>15</sub> -C <sub>20</sub> sec-alkyl)-hexahydropyrimidine-2-thione and N-methyl-N-coco-N,N-polyethyleneoxide (15 moles) ammonium chloride | .03               | 0.10                                       |
| None                                                                                                                                               | .03               | 0.34                                       |

## EXAMPLE VII

Using the experimental procedure as set forth in Example I, tests were run on mixtures of (A) N-(C<sub>7</sub>-C<sub>9</sub> sec-alkyl)-hexahydropyrimidine - 2 - thione and (B) N-methyl-N-coco-N,N-polyethyleneoxide (15 moles) ammonium chloride as corrosion inhibiting compositions for 75% phosphoric acid in contact with 1020 mild steel coupons. The tests were run at 50° C. for 48 hours. The mixtures used and the results of the tests are set forth in Table VII.

TABLE VII

| Inhibitor and Percent Inhibitor                                                                                                                  | Corrosion Rate (lb./ft. <sup>2</sup> /day) |
|--------------------------------------------------------------------------------------------------------------------------------------------------|--------------------------------------------|
| N-(C <sub>7</sub> -C <sub>9</sub> sec-alkyl)-hexahydropyrimidine-2-thione and N-methyl-N-coco-N,N-polyethyleneoxide (15 moles) ammonium chloride |                                            |
| None                                                                                                                                             | 0.34                                       |
| .02                                                                                                                                              | 0.063                                      |
| .04                                                                                                                                              | 0.0064                                     |
| .04                                                                                                                                              | 0.015                                      |
| .04                                                                                                                                              | 0.0030                                     |

## EXAMPLE VIII

Using the experimental procedure as set forth in Example I, tests were run on mixtures of (A) N-(C<sub>7</sub>-C<sub>9</sub> sec-alkyl)-hexahydropyrimidine-2-thione and (B) N-coco N,N,N-trimethyl ammonium chloride (50% active) with 75% phosphoric acid for inhibiting corrosion of 1020 mild steel coupons. The tests were run at 50° C. for 48 hours. The mixtures used and the results obtained are set forth in Table VIII.

8  
TABLE VIII

| Inhibitor and Percent Inhibitor                                                                                                     | Corrosion Rate (lb./ft. <sup>2</sup> /day) |
|-------------------------------------------------------------------------------------------------------------------------------------|--------------------------------------------|
| N-(C <sub>7</sub> -C <sub>9</sub> sec-alkyl)-hexahydropyrimidine-2-thione and N-coco-N,N,N-trimethyl ammonium chloride (50% active) |                                            |
| None                                                                                                                                | 0.34                                       |
| .02                                                                                                                                 | 0.087                                      |
| .03                                                                                                                                 | 0.0032                                     |
| .04                                                                                                                                 | 0.019                                      |
| .01                                                                                                                                 | 0.066                                      |
| .02                                                                                                                                 | 0.0054                                     |
| .03                                                                                                                                 | 0.0020                                     |

## EXAMPLE IX

Using the experimental procedure set forth in Example I, tests were run for corrosion inhibition on mild steel coupons using mixtures of (A) N-(C<sub>7</sub>-C<sub>9</sub> sec - alkyl)-hexahydropyrimidine-2-thione and (B) as a solubilizing substance or agent, a quaternary ammonium compound with concentrated (approximately 75%) phosphoric acid. Such a mixture is necessary if inexpensive mild steel is to be employed in equipment contacting concentrated phosphoric acid, as is present in the manufacture of liquid fertilizers. The efficacy of our mixtures at low concentrations makes them commercially important for use in the manufacture of liquid fertilizers containing high concentration of phosphorus because our mixtures are soluble at use concentration, are economically attractive will give little or no foaming problem, and they will not substantially stain the metal when added to the acid. The tests were run at 120° F. for 48 hours. The mixtures used and the results of the tests are set forth in Table IX.

| Inhibitor and Percent Inhibitor                                                                                                                  | Corrosion Rate (lb./ft. <sup>2</sup> /day) |
|--------------------------------------------------------------------------------------------------------------------------------------------------|--------------------------------------------|
| N-(C <sub>7</sub> -C <sub>9</sub> sec alkyl)-hexahydropyrimidine-2-thione and N-methyl-N-coco-N,N-polyethyleneoxide (15 moles) ammonium chloride |                                            |
| None                                                                                                                                             | .361                                       |
| .005                                                                                                                                             | .255                                       |
| .010                                                                                                                                             | .201                                       |
| .015                                                                                                                                             | .181                                       |
| .020                                                                                                                                             | .0985                                      |
| .025                                                                                                                                             | .0395                                      |
| .030                                                                                                                                             | .0430                                      |
| .035                                                                                                                                             | .0382                                      |
| .0075                                                                                                                                            | .154                                       |
| .010                                                                                                                                             | .109                                       |
| .0125                                                                                                                                            | .0715                                      |
| .0150                                                                                                                                            | .0625                                      |
| .0175                                                                                                                                            | .0575                                      |
| .020                                                                                                                                             | .0352                                      |
| .025                                                                                                                                             | .0274                                      |
| N,N-dioco-N,N-dimethyl ammonium chloride (75% active)                                                                                            |                                            |
| .005                                                                                                                                             | .332                                       |
| .010                                                                                                                                             | .202                                       |
| .015                                                                                                                                             | .0370                                      |
| .020                                                                                                                                             | .0204                                      |
| .025                                                                                                                                             | .0180                                      |
| .030                                                                                                                                             | .0140                                      |
| .035                                                                                                                                             | .0134                                      |
| .0025                                                                                                                                            | .346                                       |
| .0050                                                                                                                                            | .288                                       |
| .0075                                                                                                                                            | .0356                                      |
| .010                                                                                                                                             | .0220                                      |
| .0125                                                                                                                                            | .0206                                      |
| .0150                                                                                                                                            | .0150                                      |
| .0175                                                                                                                                            | .0133                                      |
| N-coco-N,N,N-trimethyl ammonium chloride (50% active)                                                                                            |                                            |
| .005                                                                                                                                             | .286                                       |
| .010                                                                                                                                             | .164                                       |
| .015                                                                                                                                             | .0307                                      |
| .020                                                                                                                                             | .0282                                      |
| .025                                                                                                                                             | .0256                                      |
| .030                                                                                                                                             | .0238                                      |
| .035                                                                                                                                             | .0216                                      |
| N,N-di(dihydroxy tallow)-N,N-dimethyl ammonium chloride (75% active)                                                                             |                                            |
| .005                                                                                                                                             | .352                                       |
| .010                                                                                                                                             | .204                                       |
| .015                                                                                                                                             | .0362                                      |
| .020                                                                                                                                             | .0182                                      |
| .025                                                                                                                                             | .0176                                      |
| .030                                                                                                                                             | .0173                                      |
| .035                                                                                                                                             | .0159                                      |

| Inhibitor and Percent Inhibitor                                                  |                                                                   |                                            |
|----------------------------------------------------------------------------------|-------------------------------------------------------------------|--------------------------------------------|
| N-(C <sub>7</sub> -C <sub>9</sub> sec-alkyl)-hexahydropyrimidine-2-thione        | N-methyl-N-coco-N,N-polyethylenoxide (15 moles) ammonium chloride | Corrosion Rate (lb./ft. <sup>2</sup> /day) |
| .015                                                                             | .015                                                              | .0415                                      |
| .020                                                                             | .020                                                              | .0270                                      |
| .025                                                                             | .025                                                              | .0221                                      |
| .030                                                                             | .030                                                              | .0188                                      |
| .035                                                                             | .035                                                              | .0173                                      |
| .040                                                                             | .040                                                              | .0153                                      |
| .045                                                                             | .045                                                              | .0151                                      |
| N-(C <sub>11</sub> -C <sub>14</sub> sec-alkyl)-N,N,N-trimethyl ammonium chloride |                                                                   |                                            |
| .015                                                                             | .015                                                              | 10 .0343                                   |
| .020                                                                             | .020                                                              | .0232                                      |
| .025                                                                             | .025                                                              | .0226                                      |
| .030                                                                             | .030                                                              | .0184                                      |
| .035                                                                             | .035                                                              | .0170                                      |
| .040                                                                             | .040                                                              | .0146                                      |
| .045                                                                             | .045                                                              | .0135                                      |
| N-(C <sub>14</sub> -C <sub>19</sub> sec-alkyl)-N,N,N-trimethyl ammonium chloride |                                                                   |                                            |
| .015                                                                             | .015                                                              | 15 .0343                                   |
| .020                                                                             | .020                                                              | .0232                                      |
| .025                                                                             | .025                                                              | .0226                                      |
| .030                                                                             | .030                                                              | .0184                                      |
| .035                                                                             | .035                                                              | .0170                                      |
| .040                                                                             | .040                                                              | .0146                                      |
| .045                                                                             | .045                                                              | .0135                                      |
| N-(C <sub>20</sub> -C <sub>22</sub> sec-alkyl)-hexahydropyrimidine-2-thione      |                                                                   |                                            |
| .015                                                                             | .015                                                              | 20 .203                                    |
| .020                                                                             | .020                                                              | .115                                       |
| .025                                                                             | .025                                                              | .0815                                      |
| .030                                                                             | .030                                                              | .0820                                      |
| .035                                                                             | .035                                                              | .0170                                      |
| .040                                                                             | .040                                                              | .0112                                      |
| .045                                                                             | .045                                                              | .00975                                     |

We claim:

1. A process for protecting metals in contact with corroding aqueous acidic solutions which comprises incorporating into said solutions a corrosion-inhibiting amount of an alkyl hexahydropyrimidine-2-thione having the formula:



wherein R is an aliphatic hydrocarbon radical having from 6 to 22 carbon atoms, and thereafter causing the said solutions to contact the metal to be protected.

2. The process of claim 1 wherein the corrosion inhibiting amount is from 10 to 50,000 parts of inhibitor per million parts of aqueous acidic solution.

3. Corrosion inhibited acidic solution compositions comprising an aqueous acidic solution and a corrosion inhibiting amount of an alkyl hexahydropyrimidine-2-thione having the formula:



Wherein R is an aliphatic hydrocarbon radical having from 6 to 22 carbon atoms.

4. The composition of claim 3 in which R is a secondary alkyl radical having from 7 to 9 carbon atoms.

5. The composition of claim 3, in which said thione is present in said solutions in an effective amount more than 10 parts per million.

6. Corrosion inhibited acidic solution compositions comprising an aqueous acidic solution and a corrosion inhibiting amount of a mixture of (A) an alkyl hexahydropyrimidine-2-thione having the formula:



wherein R is an aliphatic hydrocarbon radical having from 6 to 22 carbon atoms and (B) a quaternary ammonium compound of the formula:



wherein R<sub>1</sub> is an aliphatic hydrocarbon radical containing from 6 to 22 carbon atoms, R<sub>2</sub> is an alkyl radical containing from 1 to 3 carbon atoms, R<sub>3</sub> is a hydrocarbon radical selected from the group consisting of R<sub>1</sub>, R<sub>2</sub> and (R'O)<sub>x</sub>H wherein R' is an alkylene radical having between 2 and 3 carbon atoms, R<sub>4</sub> is a hydrocarbon radical selected from the group consisting of R<sub>1</sub>, R<sub>2</sub> and (R'O)<sub>y</sub>H provided that when R<sub>3</sub> is (R'O)<sub>x</sub>H, R<sub>4</sub> is (R'O)<sub>y</sub>H and x and y are integers having a sum between 2 and 50, and X is a halogen.

25 7. The composition of claim 6 in which the acid solution is phosphoric acid containing up to about 80% by weight phosphoric acid, and said thione and the quaternary ammonium compound are present in combination in an effective amount more than 50 parts per million.

8. The composition of claim 7 in which the proportions of said thione to the quaternary ammonium compound are from about 25% to about 75% by weight of said thione in combination with about 75% to about 25% by weight of the quaternary ammonium compound.

9. The composition of claim 8 in which said thione is N-(C<sub>7</sub>-C<sub>9</sub> sec-alkyl)-hexahydropyrimidine-2-thione and the quaternary ammonium compound is N-methyl-N-coco-N,N-polyoxyethylene (15 moles) ammonium chloride.

10. The composition of claim 9 in which the quaternary ammonium compound is N-coco-N,N,N-trimethyl ammonium chloride.

#### References Cited

##### UNITED STATES PATENTS

- |           |         |            |         |   |
|-----------|---------|------------|---------|---|
| 2,947,703 | 8/1960  | Larsonneur | 252—391 | X |
| 3,047,510 | 7/1962  | Cizek      | 252—391 | X |
| 3,294,695 | 12/1966 | Tippett    | 252—391 | X |

LEON D. ROSDOL, Primary Examiner

I. GLUCK, Assistant Examiner

60 U.S. Cl. X.R.

21—2.5; 252—149, 395

UNITED STATES PATENT OFFICE  
CERTIFICATE OF CORRECTION

Patent No. 3,457,185 Dated July 22, 1969

Inventor(s) Roy J. Betty, Robert E. Malec and Charles E. Tippett

It is certified that error appears in the above-identified patent and that said Letters Patent are hereby corrected as shown below:

Column 8, line 27, a comma should appear after the word "attractive".

Column 10, in claim 6, line 25, for "R<sub>2</sub>" read  
---R<sub>3</sub>---.

SIGNED AND  
SEALED  
JAN 20 1970

(SEAL)

Attest:

Edward M. Fletcher, Jr.  
Attesting Officer

WILLIAM E. SCHUYLER, JR.  
Commissioner of Patents

UNITED STATES PATENT OFFICE  
CERTIFICATE OF CORRECTION

Patent No. 3,457,185 Dated July 22, 1969

Inventor(s) Roy J. Betty, Robert E. Malec and Charles E. Tippett

It is certified that error appears in the above-identified patent  
and that said Letters Patent are hereby corrected as shown below:

Column 8, line 27, a comma should appear after  
the word "attractive".

Column 10, in claim 6, line 25, for "R<sub>2</sub>" read  
---R<sub>3</sub>---.

SIGNED AND  
SEALED  
JAN 20 1970

(SEAL)

Attest:

Edward M. Fletcher, Jr.

Attesting Officer

WILLIAM E. SCHUYLER, JR.  
Commissioner of Patents